

## 1

3,660,290

**LUBRICANT COMPOSITIONS**

Roland T. Schlobohm, Bethalto, Ill., assignor to Shell Oil Company, New York, N.Y.

 No Drawing. Filed Sept. 22, 1969, Ser. No. 860,035  
 Int. Cl. C10m 1/34

U.S. CL. 252—51.5 A

5 Claims

**ABSTRACT OF THE DISCLOSURE**

4-alkylphenyl-1-alkyl-2-naphthylamines and mixtures of 4-alkylphenyl-1-alkyl-2-naphthylamines with 4-alkylphenyl-2-naphthylamines are effective in improving the oxidation resistance, cleanliness and bearing performance properties of lubricant compositions.

This invention relates to a novel class of phenyl-2-naphthylamine derivatives and to lubricant compositions containing such compounds. More particularly, it relates to 4-alkylphenyl-1-alkyl-2-naphthylamines which are effective in increasing the oxidation resistance, cleanliness and bearing performance properties of lubricating oils.

Lubricants employed in high speed turbine engines, particularly modern jet aircraft engines, must be resistant to high temperature oxidative degradation. The search for additives which impart the requisite properties to such lubricating oils has led to the development of numerous oxidation inhibitors, for example phenothiazine, phenyl-1-naphthylamine, phenyl-2-naphthylamine and various diphenylamines. Certain alkylated phenyl-2-naphthylamines have also been proposed, these alkylated compounds being characterized by having one or more alkyl substituents introduced into the phenyl nucleus. With the continual development of more powerful jet engines, however, and a corresponding increase in operating temperatures, many of the prior art additives have proved to be inadequate in providing the required oxidation stability to lubricating oils. Therefore, there is a need in the art for the development of additives which will increase a lubricant's resistance to oxidative degradation and which will not form sludge, develop high acidity or viscosity, or cause the formation of deposits.

It has now been found that 4-alkylphenyl-1-alkyl-2-naphthylamines are effective in improving the oxidation resistance, cleanliness and bearing performance properties of lubricating oils. The effectiveness of these compounds is attributed in substantial part to the presence of an alkyl substituent on the naphthyl nucleus which was found to have a remarkable effect on the performance characteristics of the resulting compound.

The 4-alkylphenyl-1-alkyl-2-naphthylamines of the invention have the formula:



wherein R<sub>1</sub> and R<sub>2</sub> are alkyl groups having from 2 to 80, preferably from 2 to 16, carbon atoms. Compounds wherein the R<sub>1</sub> and R<sub>2</sub> substituents have from 4 to 12 carbon atoms and have a tertiary alkyl structure are especially advantageous for use in the present compositions, particularly those wherein R<sub>1</sub> and R<sub>2</sub> are tertiary butyl or tertiary-octyl groups.

The alkylphenyl-alkynaphthylamines of the invention can be employed in lubricant compositions either singularly, in mixtures, or in combination with alkylphenyl-2-naphthylamines which have alkyl substituents exclusively on the phenyl nucleus.

## 2

Examples of the inventive compounds include:



and the like.

It has been further found that mixtures of the hereinbefore described alkylphenyl-alkynaphthylamines with phenyl-2-naphthylamines having alkyl substituents exclusively on the phenyl ring, also impart excellent performance properties to ester base lubricant compositions; properties which in fact are superior to those which would be expected from the use of these compounds individually.

Alkylphenyl-2-naphthylamines which are suitable for use in conjunction with the additives of the invention are those having one or more alkyl substituents on the phenyl ring. Said alkyl groups may contain from 2 to 16 carbon atoms, but preferably having 4 to 12 carbon atoms and a tertiary alkyl structure. Alkylphenyl-2-naphthylamines having a single tertiary-butyl or tertiary-octyl group substituted in the 4 position of the phenyl ring have been found to be particularly effective when used in combination with the present additives. Examples of such compounds include:



and the like. Compositions wherein the ratio of the alkylphenyl-alkynaphthylamines to the non-naphthyl substituted phenyl-2-naphthylamines is 1:5 to 20:1 are very satisfactory especially those wherein the ratio is from 1:2 to 10:1.

The alkylphenyl-alkynaphthylamines of the invention are generally prepared by reacting phenyl-2-naphthylamine with a 1- or 2-alkene having from 2 to 16, or more, carbon atoms at an elevated temperature in the presence of a Friedel-Crafts catalyst, e.g., aluminum chloride. The reaction conditions largely govern the nature of the alkylated products formed. Conditions conducive to naphthyl ring substitution are described in Example 1. Employing these conditions it is possible to introduce alkyl substituents into the naphthyl nucleus thus forming the unique compounds of the present invention.

Lubricant base stocks suitable for the practice of the present invention include esters of alcohols having 1 to 20, especially 4 to 12 carbon atoms and aliphatic carboxylic acids having from 3 to 20, especially 4 to 12 carbon atoms. The ester base may comprise a simple ester (reaction product of a monohydroxyalcohol and a monocarboxylic acid), a polyester (reaction product of an alcohol and an acid, one of which has more than one func-

tional group), or a complex ester (reaction product of a polyfunctional acid with more than one alcohol, or of a polyfunctional alcohol with more than one acid). Also, excellent synthetic lubricant may be formulated from mixtures of esters, such as major proportions of complex esters and minor amounts of diesters.

Examples of suitable ester base oils are ethyl palmitate, ethyl laurate, butyl stearate, di-(2-ethylhexyl)sebacate, di-(2-ethylhexyl)azelate, ethylene glycol diluarate, di-(2-ethylhexyl)phthalate, di-(3-methylbutyl) adipate, di-(2-ethylpropyl)azelate, diisopropylolylate, dicyclohexyl sebacate, glycerol tri-n-heptanoate, di(undecyl)azelate, and tetraethylene glycol di-(2-ethyl hexanoate), and mixtures thereof. An especially preferred mixture of esters consists of about 50-80% bis(2,2,4 - trimethylpentyl)azelate and 20 to 50% 1,1,1-trimethyl propane triheptanoate.

Especially preferred esters for use as base stocks in the present invention are esters of monocarboxylic acids having 3 to 12 carbons and polyalcohols such as pentaerythritol, dipentaerythritol, trimethylolpropane and mixtures thereof. Examples of these esters are pentaerythrityl tetrabutyrate, pentaerythrityl tetravalerate, pentaerythrityl tetracaproate, pentaerythrityl dibutyratecaproate, pentaerythrityl butyratecaproate divalerate, pentaerythrityl butyrate trivalerate, pentaerythrityl butyrate tricaproate, pentaerythrityl tributyratecaproate, mixed C<sub>4</sub>-C<sub>10</sub> saturated fatty acid esters of pentaerythritol, dipentaerythrityl hexavalerate, dipentaerythrityl hexacaproate, dipentaerythrityl hexaheptoate, dipentaerythrityl hexacaprylate, dipentaerythrityl tributyratetraproate, dipentaerythrityl trivalerate tripelargonate, dipentaerythrityl mixed hexaesters of C<sub>4</sub>-C<sub>10</sub> fatty acids and trimethylol-propane heptanoate. Mixtures of pentaerythrityl and dipentaerythrityl esters of C<sub>4</sub>-C<sub>10</sub> acids are particularly advantageous base oils, and are commercially available from Hercules, Inc.

In addition to the aforementioned synthetic oils, the additives of this invention may also be incorporated in mineral lubricating oils. The mineral lubricating oil can be obtained from paraffinic, naphthenic, asphaltic or mixed base crudes and/or mixtures thereof, for example neutral oils having viscosities of from 100 to 6500 SSU at 100° F.

The alkylphenyl-alkylnaphthylamines of the invention can be incorporated into lubricant compositions in amounts of from 0.01 to 10% by weight of the total composition. Concentrations of 0.5 to 5.0% by weight are generally sufficient to impart the desired properties to lubricating oils. These concentration ranges are also applicable to mixtures of alkylphenyl-alkylnaphthylamines with alkylphenyl-naphthylamines as hereinbefore described. A preferred embodiment of the invention therefore is an ester base lubricating composition containing a total of from 0.01 to 10% by weight of a mixture of one or more 4-alkylphenyl-1-alkyl-2-naphthylamines with one or more 4-alkylphenyl-2-naphthylamines, the ratio of the former compounds to the latter being from 1:2 to 10:1.

Other additives recognized in the art to perform a particular function or functions can also be incorporated into the present compositions. These include viscosity improvers, e.g., methacrylate polymers and copolymers, additional antioxidants, corrosion inhibitors, antifoam agents, detergents and the like.

The invention will be further described by means of the following examples which demonstrate the manner of preparation and effectiveness of the inventive compounds and compositions. It should be understood, however, that these examples are given for illustrative purposes only and that the invention in its broader aspects is not limited thereto.

#### EXAMPLE I

5.36 g. (0.04 mole) of aluminum trichloride was added to 87.6 g. (0.4 mole) of phenyl-2-naphthylamine and heated to 120° C. While stirring and under a nitrogen atmosphere, 89.6 g. (0.8 mole) of diisobutylene was added dropwise to the reaction mixture over a period of one

5 hour. After the addition of the diisobutylene, the reaction mixture was heated to 148° C. over a three hour period and the temperature maintained there for an additional two hours. The reaction mixture was then allowed to cool, mixed with two volumes of benzene, poured over ice and water, washed with a 10% aqueous NaOH solution and with distilled water until neutral, after which the benzene layer was dried over CaSO<sub>4</sub>. After filtering and removal of the benzene by distillation, the crude product (146 g.) was vacuum distilled over the range of 210°/50<sub>μ</sub> to 260° C./45<sub>μ</sub>, yielding 139 g. of product. 4-tert-octylphenyl-1-tert-octyl-2-naphthylamine was isolated by means of gas chromatographic preparative techniques and was identified by infra-red spectroscopy, nuclear magnetic resonance (NMR) and elemental analysis. This compound constituted 54.99% of the reaction product.

Gas chromatographic analysis also demonstrated the presence of a mixture of two other naphthyl-substituted phenyl-2-naphthylamines constituting 15.79% of the reaction product. This mixture was separated from distilled product and identified by infra-red spectroscopy and nuclear magnetic resonance as being 4-tert-octylphenyl-1-tert-butyl-2-naphthylamine and 4-tert-butylphenyl-1-tert-octyl-2-naphthylamine.

#### EXAMPLE II

To illustrate the ester base compositions of the invention, Compositions II, III, V, VI, VIII and XI were formulated as shown in Table I, and thereafter compared to Compositions I, IV, IX and X not in accordance with the invention, by means of one or more of the test procedures hereinafter described.

TABLE I

| Composition: | Base oil | Phenyl-2-naphthylamine | Additive, percent weight           |            |
|--------------|----------|------------------------|------------------------------------|------------|
|              |          |                        | 4-tert-octylphenyl-2-naphthylamine | Additive A |
| I            | W        | -----                  | 1.5                                | -----      |
| II           | W        | -----                  | 1.5                                | 1.84       |
| III          | W        | -----                  | 1.5                                | 1.84       |
| IV           | X        | -----                  | 1.5                                | 1.84       |
| V            | X        | -----                  | 1.5                                | 1.84       |
| VI           | X        | -----                  | 1.5                                | 1.84       |
| VII          | Y        | -----                  | 1.5                                | 1.84       |
| VIII         | Y        | -----                  | 1.5                                | 1.84       |
| IX           | Z        | 1.0                    | 1.5                                | 1.84       |
| X            | Z        | -----                  | 1.5                                | 1.84       |
| XI           | Z        | -----                  | 1.5                                | 1.84       |

<sup>1</sup> Equal molar concentrations equivalent to 1.0% w. phenyl-2-naphthylamine in base oil.

#### Additives

Additive A: 4-tert-octylphenyl-1-tert-octyl-2-naphthylamine

Additive B: Mixture of 4-tert-octylphenyl-1-tert-octyl-2-naphthylamine, 4-tert-butylphenyl-1-tert-octyl-2-naphthylamine and 4-tert-octylphenyl-1-tert-butyl-2-naphthylamine with 4-tert-octylphenyl-2-naphthylamine, Ratio of alkylphenyl-alkylnaphthylamines to 4-tert-octylphenyl-2-naphthylamine is approximately 3 to 1.

#### Base Oils

Base Oil W: Mixed C<sub>4</sub>-C<sub>10</sub> acid esters of pentaerythritol and dipentaerythritol containing 0.17% w. of phosphorus extreme pressure agents, 0.1% w. of triazole corrosion inhibitors, 0.25% w. of a copolymeric dispersant, 1.5% w. of an amine antioxidant, 0.02% of a dibasic acid corrosion inhibitor and 10 p.p.m. silicone fluid antifoamant.

Base Oil X: Base Oil W minus the copolymeric dispersant plus 2.0% w. additional phosphorus extreme pressure agent.

Base Oil Y: Base Oil X minus the dibasic acid corrosion inhibitor and 1.0% of phosphorus extreme pressure agent plus 0.5% w. of a triazine oxidation inhibitor and an additional 0.5% of the amine antioxidant.

Base Oil Z: Mixed C<sub>4-10</sub> acid esters of pentaerythritol and dipentaerythritol containing 0.2% w. phosphorus extreme pressure agent and 0.5% w. of a triazole corrosion inhibitor.

### EXAMPLE III

To demonstrate the advantages of the present compositions in respect to oxidation stability and high temperature bearing performance, Compositions IV, V and VI, all prepared from Base Oil X, were subjected to a Bearing Rig Test under the very severe Type 2½ conditions. The results of these tests are shown in Table II. The Bearing Rig Test is described in Military Specification MIL-L-23699.

TABLE II

| Bearing rig test, 80 hours type 2½      | Composition— |       |       |
|-----------------------------------------|--------------|-------|-------|
|                                         | IV           | V     | VI    |
| Overall demerit rating.....             | 69           | 38.6  | 28.2  |
| Filter deposits, grams.....             | 0.43         | 0.45  | 0.45  |
| Viscosity change, 100° F., percent..... | 1,705        | 863   | 406   |
| Acid number change.....                 | 5.76         | 4.11  | 4.22  |
| Oil consumption, milliliter.....        | 4,470        | 3,987 | 5,879 |

From the above data it is evident that Compositions V and VI of the invention have outstanding properties in respect to overall cleanliness and viscosity change as compared to Composition IV which contains an equal molar concentration of a phenyl-2-naphthylamine having no alkyl substituents on the naphthyl ring. It is indeed surprising that the addition of an alkyl substituent on the naphthyl nucleus (Additive A) would bring about such a significant improvement in the effectiveness of the inventive compounds. Moreover, it is equally remarkable that Composition VI, which contains a combination of the additives of the invention with the additive employed in Composition IV, has an overall demerit rating superior to that of either Compositions IV or V containing the additives individually, i.e., a total demerit rating of 28.2 as compared to 69 and 38.6 respectively.

### EXAMPLE IV

A further indication of the stability of the compositions of the invention was obtained by subjecting samples of Compositions VII and VIII to the Alcor High Temperature Deposition Test. Basically this test involves circulation of aerated oil over a heated deposition tube. The temperature of the tube is controlled at 525° F. on the inlet side and reaches 650 to 700° F. at the outlet end of the tube. The temperature profile of the tube is measured at the start and shortly before the end of the test. These temperature profiles and the tube deposits per unit length are used to determine the performance of the oil. The critical temperature is that temperature at which deposits begin to significantly affect the heat transfer characteristics of the oil. A temperature of about 600° F. is considered to be very satisfactory. The overall deposit rating is obtained from a combination of the visual deposit rating of the tube, the tube deposit weight and the filter deposit weight. An overall rating of less than 50 is considered very good, a rating of below 15 is considered exceptional. A detailed description of this test is given in "Proceedings of the USAF-Southwest Research Institute Turbine Lubrication Conference," September 13-15, 1966, Southwest Research Institute, San Antonio, Texas, page 152. Test results are shown in Table III.

TABLE III

|                                         | Composition— |       |
|-----------------------------------------|--------------|-------|
|                                         | VII          | VIII  |
| Alcor high temperature deposition test  |              |       |
| Critical temperature, ° F.....          | 630          | 640   |
| Tube deposit rating, demerits.....      | 10           | 5.8   |
| Tube deposits milligrams.....           | 2            | 5.1   |
| Filter deposits, milligrams.....        | 31           | 10.8  |
| Oil consumption, milliliters.....       | 225          | 125   |
| Viscosity change, 100° F., percent..... | 20.3         | 30.6  |
| Acid number change.....                 | +0.18        | +0.22 |
| Overall deposit rating.....             | 21.5         | 10.9  |

The foregoing results indicate that Composition VIII of the invention, has a significantly less tendency to form deposits than Composition VII which is prepared from the same base oil as Composition VIII but contains an alkylated phenyl-2-naphthylamine not in accordance with the invention.

### EXAMPLE V

In order to further evaluate the antioxidation and anti-corrosion properties of the present compositions, a series of Corrosion and Oxidation Stability Tests were run in accordance with the procedures set forth in Military Specification MIL-L-23699. In addition, Compositions IX, X, and XI were subjected to a Micro-Air Oxidation Test. In this test, air at the rate of 30 ml./min. was passed through a 20 g. sample of the test lubricant which was maintained at a temperature of 425° F. The results of the test are expressed as oxidation life of the lubricant, which is defined as the time required for the adsorption of 3 millimoles of oxygen per gram of oil sample. The results of the Micro-Air Oxidation Test and the Corrosion and Oxidation Stability Test are shown in Table IV.

TABLE IV  
[Corrosion and oxidation stability, 400° F., 72 hours]

|                                         | Composition— |       |       |
|-----------------------------------------|--------------|-------|-------|
|                                         | I            | II    | III   |
| Weight change of specimens:             |              |       |       |
| Mg.....                                 | -0.01        | +0.01 | +0.01 |
| Al.....                                 | -0.03        | -0.01 | -0.01 |
| Cu.....                                 | -0.13        | -0.10 | -0.16 |
| Fe.....                                 | -0.02        | +0.01 | +0.01 |
| Ag.....                                 | -0.10        | -0.11 | -0.09 |
| Viscosity change, 100° F., percent..... | 23.4         | 37.8  | 15.2  |
| Acid number change.....                 | 0.81         | 1.43  | 1.54  |
| Sludge, mg./100 ml.....                 | 19.0         | 2.0   | 3.0   |

#### Micro-air oxidation test, 425° F.

|                            | Composition— |    |    |
|----------------------------|--------------|----|----|
|                            | IX           | X  | XI |
| Oxidation life, hours..... | 70           | 67 | 75 |

It is evident from the Corrosion and Oxidation Test results, that Compositions II and III of the invention have surprisingly less tendency to form sludge than Composition I which contains a molar equivalent of an additive not in accordance with the invention. In the Micro-Air Oxidation Test, Composition XI of the invention had a significantly longer oxidation life than either Composition IX containing phenyl-2-naphthylamine, or Composition X containing an equivalent amount of a phenyl-2-naphthylamine having an alkyl substituent on the phenyl ring alone.

I claim as my invention:

1. A lubricant composition consisting essentially of a major amount of lubricating oil and an oxidation-inhibiting amount of a mixture of at least one 4-alkylphenyl-1-alkyl-2-naphthylamine with at least one 4-alkylphenyl-2-naphthylamine wherein said alkyl substituents have up to 16 carbon atoms and are tertiary alkyl substituents and the ratio of said alkylphenylalkylnaphthylamines to the alkylphenyl-naphthylamines is from 1:2 to 10:1.

2. The composition of claim 1 wherein the oxidation inhibiting mixture is present in the amount of from 0.01 to 10% by weight.

3. The composition of claim 1 wherein the lubricating oil is an ester of a monocarboxylic acid having 3 to 12 carbon atoms and a polyhydroxy compound selected from the group consisting of pentaerythritol, dipentaerythritol, trimethylolpropane and mixtures thereof.

4. The composition of claim 3 wherein all of the alkyl substituents are selected from the group consisting of tertiary-butyl and tertiary-octyl.

5. The composition of claim 4 wherein the ester lubricating oil is a mixed  $C_{4-10}$  acid ester of pentaerythritol and dipentaerythritol and the oxidation-inhibiting mixture is a mixture of 4-alkylphenyl-1-alkyl-2-naphthylamines with 4-tert-octylphenyl-2-naphthylamine.

## References Cited

## UNITED STATES PATENTS

|           |        |              |            |
|-----------|--------|--------------|------------|
| 2,009,480 | 7/1935 | Craig        | 252—50     |
| 3,052,632 | 9/1962 | Loeffler     | 252—51.5 A |
| 3,121,691 | 2/1964 | Eickemeyer   | 252—50 X   |
| 3,505,225 | 4/1970 | Wheeler      | 252—50 X   |
| 3,509,214 | 4/1970 | Braid et al. | 252—50 X   |

## FOREIGN PATENTS

|           |        |        |        |
|-----------|--------|--------|--------|
| 1,429,495 | 1/1966 | France | 252—50 |
|-----------|--------|--------|--------|

DANIEL E. WYMAN, Primary Examiner

W. J. SHINE, Assistant Examiner

U.S. Cl. X.R.

252—50, 390, 401